

Patented Oct. 31, 1933

1,933,490

# UNITED STATES PATENT OFFICE

1,933,490

## ZINC ALLOY AND CERTAIN ARTICLES MADE THEREFROM

Leland E. Wemple, Chicago, and John R. Daesen,  
Oak Park, Ill.

No Drawing. Application April 26, 1932  
Serial No. 607,664

3 Claims. (Cl. 75—1)

Our invention relates to new and useful alloys of zinc whose advantages will be herein-after set forth, and to certain articles produced from such alloys. The alloys are prepared by adding to 100 parts of zinc from .025 to .245 part of copper and from .001 to .245 part of silver.

In our United States Letters Patent No. 1,789,854 we have claimed an alloy consisting of 10 100 parts zinc, .25 to 2 parts of copper, and silver in an amount less than the copper used. We have now found that some of the advantages of such invention may be obtained if the proportion of copper is reduced to within the range of 15 .025 to .245 part and silver is present from .001 to .245 part, and regardless of whether the silver is less than, equal to or greater than the amount of copper.

An alloy produced in accordance with our 20 invention may be rolled into sheets or strips whose surface can be brought to an attractive condition by polishing, the polished surface maintaining its lustre, and which have a higher tensile strength than sheets or strips rolled from 25 zinc or known zinc base alloys, and such new sheets or strips are capable of acquiring increased strength by subsequent forming operations. At the same time the natural advantages of the zinc are not reduced, in any event, to any appreciable 30 or substantial extent. The low proportion of copper used renders the alloy much more ductile so that it may more readily be used for the manufacture of articles by extrusion and deep drawing. The use of silver within the proportions stated serves to toughen the alloy and thereby broaden its field of usefulness.

The zinc used in the production of the alloy 40 may be a high grade zinc but for practical purposes we prefer to use the lower grades of commercial slab zinc or spelter which should, however, not contain ingredients which detrimentally affect the alloy. The presence of more than .6% of cadmium or .04% of iron renders the zinc too brittle for rolling into thin gauges. The presence of even a small trace of aluminum causes the alloy, after rolling, to develop cracks and to disintegrate. For practical purposes we prefer to use a grade of spelter known in the trade as "intermediate", whose maximum iron content is .03%, maximum lead content .2%, and maximum cadmium content .5%, but not more than a total of .5% of all such metals, and which is substantially free from aluminum and magnesium.

55 We may, however, use to advantage the grade

of spelter known as "brass special" or the grade known as "high grade" or electrolytic zinc.

The exact proportion of copper and of silver will depend upon the particular qualities of the alloy to be produced and also upon the various conditions of the process, for instance, rolling, to which the alloy is to be subjected. The particular proportions may easily be adjusted by simple experiment until the correct proportion suitable for the desired alloy is determined.

### Example I

Approximately 10,000 lbs. of slab spelter, electrolytic grade, containing 99.9% zinc, a trace of iron, cadmium and lead, are charged into a coal-fired tank furnace and the temperature of the furnace maintained at 825-850° F. When the slabs of spelter are completely melted forming a bath of molten zinc, the dross is carefully skimmed off and 12 lbs. of copper in the form of scrap sheet or wire are added and stirred into the molten metal; then 3 1/4 lbs. of silver are added in the form of pellets and stirred into the bath of molten metal. After both the copper and silver are thoroughly incorporated into the zinc, the molten alloy is cast into plates suitable for rolling. After storage in warming ovens in the manner usual with ordinary zinc, these plates are passed through roughing and finishing rolls in a like manner as with ordinary zinc to form sheets or strips.

The alloy thus produced rolled in sheets to a thickness of .0625" assays approximately as follows, and possesses physical properties as listed below. For purposes of comparison, the assays and physical properties of pure electrolytic zinc treated in the same manner are also listed below:

| Assay                                          | Alloy           | Electrolytic zinc |
|------------------------------------------------|-----------------|-------------------|
| Percent                                        |                 | 95                |
| Copper.....                                    | .12.....        | None.....         |
| Silver.....                                    | .03.....        | None.....         |
| Iron.....                                      | .006.....       | .006.....         |
| Lead.....                                      | Trace.....      | Trace.....        |
| Cadmium.....                                   | Trace.....      | Trace.....        |
| Zinc.....                                      | Balance.....    | Balance.....      |
| <i>Physical properties of rolled sheets</i>    |                 |                   |
| Gauge.....                                     | .0625"          | .0625"            |
| Hardness, Rockwell.....                        | 80.....         | 68.....           |
| Tensile strength per sq. in. across grain..... | 32,000 lbs..... | 21,900 lbs.....   |
| Dynamite ductility.....                        | 430.....        | 465.....          |

### Example II

1,000 lbs. of commercial electrolytic spelter 110

containing .01% iron, a trace of lead and a trace of cadmium, are melted in an oil-fired tank furnace. When the zinc is thoroughly molten, there are added 1.35 lbs. of copper in the form of a sheet and .68 lbs. of silver in the form of metallic silver. The ingredients are allowed to thoroughly mix and the alloy is then cast in slabs 1" thick which are rolled into sheets of .04" gauge.

10 The finished sheets assay approximately as follows and possess the physical properties indicated:

| 15                                          | Assay                                     |             | Alloy       | Electrolytic zinc |
|---------------------------------------------|-------------------------------------------|-------------|-------------|-------------------|
|                                             | Percent                                   |             |             |                   |
| 16                                          | Iron                                      | .01         | None        |                   |
| 17                                          | Copper                                    | .135        | None        |                   |
| 18                                          | Silver                                    | .068        | .003        |                   |
| 19                                          | Lead                                      | Trace       | Trace       |                   |
| 20                                          | Cadmium                                   | Trace       | Trace       |                   |
| 21                                          | Zinc                                      | Balance     | Balance     |                   |
| <i>Physical properties of rolled sheets</i> |                                           |             |             |                   |
| 22                                          | Gauge                                     | .04"        | .04"        |                   |
| 23                                          | Tensile strength per sq. in. across grain | 29,200 lbs. | 22,100 lbs. |                   |
| 24                                          | Rockwell hardness                         | 60          | 60          |                   |
| 25                                          | Dynamic ductility                         | 70          | 440         |                   |
|                                             |                                           | 460         |             |                   |

It will be noted that the hardness of our alloy is substantially greater by the Rockwell scale than ordinary rolled zinc and that the tensile strength of our alloy is appreciably greater than that of electrolytic zinc. At the same time the ductility of the alloy, as indicated by the readings on the dynamic testing machine and on the bending machine, shows that the increase in hardness and tensile strength has been obtained without any material change in ductility.

Having thus described the invention, what we claim as new and desire to secure by Letters Patent of the United States is:

We claim:

1. As a composition of matter, an alloy consisting principally of zinc, containing from .025 to .245 part of copper and from .001 to .245 part of silver.

2. A tertiary zinc-base alloy consisting of 100 parts of zinc, .025 to .245 part of copper, and .001 to .245 part of silver.

3. As a new article of manufacture, a mechanically worked zinc product made of a zinc-base alloy composed of zinc 100 parts, copper .025 to .245 part, and silver from .001 to .245 part.

LELAND E. WEMPLE.  
JOHN R. DAESEN.